

Sept. 27, 1938.

E. BLÜMNER

2,131,308

## PRODUCTION OF COLLOIDAL FUEL

Filed Jan. 18, 1936



## UNITED STATES PATENT OFFICE

2,131,308

## PRODUCTION OF COLLOIDAL FUEL

Erwin Blümner, London, England

Application January 18, 1936, Serial No. 59,753  
In Great Britain January 21, 1935

3 Claims. (Cl. 44—8)

This invention relates to the production of true colloidal fuel and low boiling-point hydrocarbons from solid bituminous fuels, more particularly coal, and provides a process and an apparatus for subjecting suspensions of such solid fuels, in pulverized state, in hydrocarbon oils to heat treatment under pressure, accompanied by mechanical trituration and grinding.

According to the present invention, solid bituminous fuel, such as bituminous coal, which is pulverized so as to be capable of passing through a 150- to 200-mesh screen, is suspended in crude oil, fuel oil or other high-boiling hydrocarbon oils, and is then heated up to about 450° C., under a pressure exceeding 20 atmospheres, under which treatment the bituminous constituents of the fuel undergo conversion between 270° and 400° C. This change is accompanied by the formation of gas and the evolution of steam and at the same time the viscosity of the mass increases, but diminishes again as the temperature continues to rise, and finally falls to a level that is below that of the original solid fuel oil suspension.

During the performance of the process of the present invention the suspension is temporarily emulsified, the reaction products of the bitumen passing into solution in the oil and even the finest pores and channels in the residual carbonaceous mass becoming filled with oil instead of with bitumen, thus forming a soft and readily triturable mass which, if sufficiently manipulated, assumes such a finely divided condition that a colloidal solution of carbonaceous matter in oil is obtained. By this means bituminous fuels, such as bituminous coal, can be converted into the colloidal condition in a relatively simple manner without high working costs, an operation which cannot be economically effected by mechanical means alone.

A point of special importance in carrying out the present process is that the mechanical treatment of the solid fuel oil suspension should be performed simultaneously with the progressive conversion due to the heat treatment under pressure; firstly, in order to produce a most intimate emulsification of the carbonaceous substance with the oil, and secondly, to effect extreme disintegration and grinding of the residual carbonaceous skeleton to colloidal fineness, immediately after the emulsification phase.

Simple though the herein-described operations may seem, the phenomena of molecular conversion occurring during said process are, nevertheless, exceedingly complex. The reaction products

of the coal bitumen, for example, are not low-temperature tars and, in any event, are comparable only with tars obtained by steam distillation in vacuo. The finely divided residual carbon dispersed in the oil is not coke, but a carbonaceous substance—containing the ash constituents, of course—which is comparable, to some extent, with the residues from the extraction of coal, though this latter process, being usually performed with solvents of low boiling point, does not—nor can it—ever lead to the complete extraction of the bitumen.

In the final heating state of about 400 to 450° C., the solution of bitumen in oil which also contains the colloidal carbonaceous matter is subjected to a moderate cracking treatment, accompanied by continuous trituration. During this treatment, as yet unidentified molecular reactions and migration of hydrogen between the oil and the coal hydrocarbons occur. It has been ascertained that the bituminous matter in coal for example, furnishes considerably larger yields of benzine when treated in accordance with the present invention than when treated by itself, even when allowance is naturally made for the benzine attributable to the oil vehicle itself.

The apparatus designed for carrying out the improved process is illustrated diagrammatically and by way of example on the accompanying drawing in which Figure 1 is in its left-hand portion (larger than the right-hand half of the sheet) a vertical section through that apparatus, and in its remaining portion, in the right-hand half of the sheet, a side view of certain additional members, all as fully described hereinafter, and Figure 2 is a horizontal section through a portion of one of the vertical cylinders visible in Fig. 1, drawn to a considerably enlarged scale.

On the drawing, 1 denotes a storage vessel or receptacle for the coal-oil suspension which enters into the vessel 1 through a tube 1<sub>a</sub> and which is pumped by means of a high-pressure pump 2 from the vessel 1 and through pipes 3 and 4 into the serpentine tube 4<sub>a</sub> in the interior of a heat-exchanger 5 from which said suspension passes through a pipe 6 into a vertical cylindrical heating vessel 7<sub>a</sub> in which the suspension is heated to about 100° C. There is a plurality of such vessels (six in the example shown, viz 7<sub>a</sub>, 7<sub>b</sub>, 7<sub>c</sub>, 7<sub>d</sub>, 7<sub>e</sub>, 7<sub>f</sub>) assembled in a masonry-furnace 8 having flues 8<sub>a</sub> in which said vessels are located and through which heating gases, maybe furnace gases or waste gases, (for example coming from the gas tube 28<sub>a</sub>) are con-

5

10

15

20

25

30

35

40

45

50

55

ducted so as to heat the said vessels to about the temperature stated. All vessels 7 . . . are of equal construction. Each comprises, besides the vessel 7 . . . proper, a cylindrical rotary insertion 9 filling the vessel to such an extent that only a narrow tubular passage 10 remains through which the suspension must pass. Each insertion 9 is firmly connected with an upper shaft 12 turned by any suitable means so as to 10 rotate in turn the insertion 9.

The tubular space or passage between the stationary vessel 7, and the rotary insertion 9 is subdivided into a plurality of parallel compartments, say six, by vertical members 11 (Fig. 2) 15 of about shoe-like transverse section which contact with the inner surface of the respective vessel 7 and are secured to elastic strips 13 affixed to the outer surface of the appertaining member 9. The suspension forced through the tubular 20 passage flows now not only vertically, but is also rotated on its way through said passage, and owing to the suitably chosen shape of the members 11 the particles contained in the suspension are very finely triturated.

25 14 denotes a foot-bearing for the rotary insertion 9. There is, of course, provided a foot bearing 14 for every insertion.

Between each two vessels 7 is located in the furnace 8 a narrow cylinder 16, the upper end of which is connected with one of the adjacent vessels 7a by means of a bent pipe 15 by which the contents of the vessel 7a treated therein is conducted into the second vessel (7b). The cylinder 16 is not located in a flue and, therefore, not heated by hot gases. The cylinder 16 receives the entire contents of the vessel 7a, i. e. the liquid, the vapor and the gas, which components of the suspension are separated in the said cylinder.

In each cylinder 16 is a long vertical float 17 connected at its upper end with an outer automatically acting needle valve 18 regulating the height of the level in the respective cylinder, independent of the pressure in the cylinder. If the formation of gas increases and, therefore, the level of the liquid in the cylinder is pressed below a certain normal height, the float 17 opens the appertaining needle valve 18 whereupon the gas and the vapor escape into a pipe 19 through which they pass to an expansion vessel 20. When then the liquid in the cylinder 16 again rises, the float 17 is lifted by it and the valve 18 is closed.

float 17 is lifted by it and the valve 18 is closed. It is a very important condition and a high advantage of my new process and apparatus, that there comes gas free coal-oil fluid only from one heated cylinder 1 to the next one over the cylinders 16 through the pipes 15 and 21.

60 All cylinders 16 are connected up in parallel to the vessel 20, but the vessels 1 (7a-7r) are connected up in series, and the last of these vessels (7r) is connected with the vessel 20 by the intermediary of the last cylinder 16 and by a pipe 22 extending into the vessel 20 from below to about into the middle portion of said vessel where it is attached to a so-called expansion colloidal mill comprising a stationary disk 23 firmly connected with the pipe 22, and a rotary disk 24 connected

with a vertical shaft 25 by which it is rotated. The two disks are polished and are made of a specially selected kind of steel. The shaft 25 is provided with a weight 26 so as to exert a corresponding pressure upon the shaft 25, or upon the two disks 23 and 24 and the composition entering between them and being acted on between them. The object of said weight is mainly to maintain the pressure in the system, or to regulate the pressure exerted by the pump 2. The supply of heat to the heating chambers in the masonry-furnace 8 is so regulated that the highest heat is in the first flue (8a) and the lowest temperature is in the last flue containing the vessel 7. Owing to a certain reduction of pressure in the mill 23, 24 another fall of temperature takes place in the chamber or vessel 20, the final temperature of the product being about 260° C., whereas the initial temperature had amounted to 450° C.

All hydrocarbons evaporating below 260° C. distill through the pipe 27 into the fractional distillation column 28. The benzinnes are withdrawn through the pipe 29 and are condensed in the condenser 30, wherefrom the condensed benzine 25 is conducted through the pipe 31 into a separator 32 in which water and gas are separated from the benzine, and from which the benzine flows through the tube 32b to a not shown benzine storage vessel and the water is conducted away through the tube 32c, as indicated. The gas-tube 32a is connected with the gas-tube 28a of the distillation column 28 of the plant.

The hot, true colloidal fuel collecting on the bottom of the vessel 20 passes through a pipe 33 into the heat-exchanger 5 containing the serpentine tube 4, and flows from the heat-exchanger 5, through a pipe 34 into a collecting tank (not shown).

I claim:

1. A process for the production of colloidal fuel comprising pulverizing solid bituminous fuel and suspending the same in high-boiling hydrocarbon oil, successively subjecting the mixture to heat and pressure in step by step operations with the heat progressively reduced, removing gas and steam between the heating steps, and driving off remaining gases to form a true colloidal fuel of the residue. 45

2. A process for the production of colloidal fuel comprising pulverizing solid bituminous fuel and mixing the same with high-boiling hydrocarbon oil to provide a suspension, successively subjecting the suspension to heat and pressure while imparting a whirling motion thereto and alternately cooling the suspension, the steps of heating being at progressively reduced temperatures and gas and steam being withdrawn during each cooling step, and then allowing the suspension to expand and grinding the treated suspension and removing the remaining gas to form a true colloidal fuel of the residue. 50 55 60

3. The process set forth in claim 2 wherein the suspension is subjected to trituration during the whirling motion as it is successively heated.

successively heated.